

Patented Oct. 21, 1950

1,779,258

## UNITED STATES PATENT OFFICE

FRANK A. McDERMOTT, OF CLAYMONT, AND FOREST J. FUNK, OF WILMINGTON, DELA-  
WARE, ASSIGNORS TO E. I. DU PONT DE NEMOURS & COMPANY, OF WILMINGTON,  
DELAWARE, A CORPORATION OF DELAWARE

## RESISTANT MATERIAL

No Drawing.

Application filed April 3, 1925. Serial No. 20,425.

This invention relates to resistant material and more particularly to fabric so treated as to be resistant to the growth of fungus and, preferably, waterproof and also resistant to acid and to fire. The present fabric finds particularly advantageous use as material for mine ventilating tubing, although not confined to such use. It is an object of the invention to provide material having the indicated, and other, desirable characteristics; it is also an object to provide mine ventilating tubing having such characteristics, and it is a further object to provide a process for the production of such material. To these ends, and also to improve generally upon materials and tubing of the character indicated, the invention consists in the various matters hereinafter described and claimed.

20 A material for mine ventilating tubing has heretofore been described, such material consisting of fabric coated with a rubber film having fungicidal and acid-resistant substances therein, U. S. Patent No. 1,432,585, 25 Abraham, October 17, 1922, and such material is, in many instances, satisfactory. However, further experience has indicated that such material is susceptible of improvement, both as to the incorporation of the fungicide and 30 the character of the fungicide. In particular, it has been found highly desirable to take special precautions against the possibility of mold growth in the fabric, to make the coating tough, and to use fungicides of somewhat different character from those suggested by Abraham. The present invention comprises a coated fabric embodying advantageous features of the type suggested.

In accordance with the present invention, 40 the fabric itself, prior to coating, is thoroughly impregnated with fungicide, such a fungicide being used that it may be applied in a solution that will thoroughly and actually penetrate the fibers of the fabric, leaving an ample deposit of fungicide actually in the fibers. This treatment guards against the possibility of the rubber coating not sufficiently penetrating the fabric to cover all the fibers thoroughly. The rubber coating 45 composition is colloidal rather than a true

solution and the size of the compound particles is so great that the solution will not readily actually penetrate, and wet, the cotton fibers. When they do not, even though the rubber coating itself carry a fungicide, the fabric itself may not be fully protected. Furthermore, since the rubber coating primarily protects but the surface of the fabric, it does not appreciably retard the germination of spores reaching the fabric through slight initial defects, or cracks subsequent to manufacture, which may occur in the coating. Again, the treating of the fabric itself with fungicide gives to fabric coated upon but one side usefulness in locations where 60 waterproofing is called for upon but one side while protection from fungus is required upon both.

The impregnating fungicides used are preferably slightly water-soluble heavy metal salts of organic acids, having antiseptic properties. Examples of these are zinc salicylate and zinc benzoate, but others will, of course, suggest themselves. However, in using others, suitable caution should be observed; for example, copper salts, on account of their oxygen-carrying possibilities, should, if used in connection with a coating of rubber, be used with care, and if silver salts are used due regard must be given to their cost. A high water solubility is best avoided as it results in rapid removal of the fungicides by mine waters; but some water solubility is desirable: samples under test show that water-soluble salts, dissolving into the water surrounding the sample inhibit the germination of mold spores in a zone immediately surrounding the sample. In other words, a water-soluble fungicide will diffuse into water when the treated fabric is dampened, and suppress the growth of molds. A water-insoluble fungicide will not do this, although it may be effective in preventing the growth of the mold in the portion of the material—e. g., the coating—in which it is included. Where the coating is of rubber, such salts as have any material deteriorating effect on rubber should preferably be avoided.

The manufacture of the material may be

55

60

65

70

75

80

85

90

95

carried out as follows:—A 2½% (by weight) solution of zinc salicylate is prepared by dissolving the salt in water. The fabric, for example duck, a drill, or an Osnaburg, 5 preferably more than eight ounces to the square yard in weight, is soaked in this solution in any suitable container, preferably by passing the material several times through the solution until it is thoroughly saturated, 10 for example has absorbed substantially its own weight of solution. After impregnation, the material should not be mangled but should be placed in a suitable dryer directly from the bath. Conveniently, a large drum 15 heated on the inside with steam coils may be used as a dryer. This treatment gives substantially 2½% of zinc salicylate in the fabric, based on the weight of the fabric. Generally speaking, at least 1% of zinc 20 salicylate, based on the weight of the fabric, is desirable for beneficial effect, while the maximum percent usable will be governed by appearance, method of application, and like factors.

25 The impregnation completed, a suitable rubber composition is applied, to one or both sides of the fabric, preferably both, the early applications of the composition being driven into the fabric, so well as may be, and then 30 a sufficient quantity spread on the fabric to render the material waterproof. The early applications may be applied by a two-roll type of "impregnator" so-called, and the later ones by means of a regular spreading 35 machine until the desired weight of coating is obtained to render the material waterproof.

By way of example, a suitable composition (parts by weight) may be as follows:—

|                 |        |
|-----------------|--------|
| 40 Crude rubber | 25     |
| Litharge        | 8      |
| Sulphur         | ¾      |
| Barytes         | 52 3/4 |
| Zinc salicylate | 2      |
| 45 Pine tar     | 4      |
| Paraffin        | 7 1/2  |

It will be understood that the above is but a specimen formula, and that it may be considerably varied without departure from the invention. For instance, the percentage of rubber can be varied from a very small percentage up to almost 100%, the litharge and sulphur varying with the rubber. The zinc 50 salicylate, or the pine tar, or both, can be omitted if it should for any reason be desirable, the omitted fungicide being replaced by an equal amount of barytes. The paraffin may range from 5 to 10% of the total weight 55 of the ingredients of the composition. The zinc salicylate to be appreciably beneficial, should be used to the extent of at least 1% of the composition, and any greater amount desired may be used so long as the physical 60 characteristics of the coating, its ease of ap-

plication, and the like, are not objectionably affected. As to the pine tar, assuming it to have a phenol coefficient of 1, at least 1% should be used for substantial effect, the maximum amount usable depending on considerations such as those mentioned in connection with the zinc salicylate. In using the composition it is dissolved in an equal weight of gasoline.

After the coating, tale is applied to the 75 coating to prevent sticking, and then the material is festooned in a suitable vulcanizing chamber and the heater closed. In vulcanizing, the temperature is carried to about 250° F. in the first hour and this temperature is maintained for about two and one-half hours, completing the vulcanizing. This completes the manufacture of the material.

In making mine ventilating tubing, the 85 material may be cut to size and made up in the usual ways of the art, and where material coated upon but one side is used such side should constitute the outer or exterior side of the tubing. The paraffin in the composition gives it resistance to the dilute acids 90 present in mines, such as 3% sulphuric acid drip, while the barytes increases its fire resistance. For the paraffin may be substituted other chemically inert substances, 95 preferably of similar physical consistency, and for the barytes may be substituted such materials as asbestos, flour, silex, lithopone, etc. Should the increased acid or fire resistance be deemed uncalled for in any particular circumstance, the acid resistant, or the fire resistant, or both, may be omitted to meet the particular desires of the user of the material. If desired, the fabric itself 100 may be treated with pine tar, or similar fungicide, but the slightly water-soluble salts are preferable as above indicated.

We claim:

1. As an article of manufacture, fungus 110 resistant material comprising a fabric base, the fibers of the fabric being impregnated with an organic salt of zinc having substantial fungicidal properties in an amount equal to at least 1% based on the weight of the fabric and a water solubility approximately 115 that of zinc salicylate and zinc benzoate, and said base being coated with a waterproofing composition also containing said salt.

2. As an article of manufacture, fungus 120 resistant material comprising a fabric base, the fibers of the fabric being impregnated with zinc salicylate, and having a coating of vulcanized rubber.

3. As an article of manufacture, fungus 125 resistant material comprising a fabric base, the fibers of the fabric being impregnated with zinc salicylate, in an amount equal to at least 1% based on the weight of the fabric, and having a coating of vulcanized rubber 130

containing fungus, fire, and acid resistant ingredients.

4. As an article of manufacture, fungus resistant material comprising a fabric base, the fibers of the fabric being impregnated with a heavy metal salt of an organic acid having substantial fungicidal properties and a water solubility approximately that of zinc salicylate and zinc benzoate, and said base being coated with a waterproofing composition.
5. As an article of manufacture, fungus resistant material comprising a fabric base, the fibers of the fabric being impregnated with a heavy metal salt of an organic acid having substantial fungicidal properties and a water solubility approximately that of zinc salicylate and zinc benzoate, and said base being coated with a waterproofing composition primarily of rubber and being strongly resistant to the action of fungi.
6. The process of producing a fungus resistant material which comprises impregnating the fibers of a fabric with a fabric-wetting solution of a slightly water-soluble organic salt of zinc having substantial fungicidal properties, depositing the fungicide in the fibers of the fabric, and coating the fabric with a rubber waterproofing composition.
7. The process of producing a fungus-proof and waterproof rubber-coated fabric which comprises impregnating the fibers of a fabric with a solution containing not less than 1% by weight based on the fabric, of a slightly water soluble non-volatile heavy metal salt of an organic acid having substantial fungicidal properties, heating to evaporate the solvent and to deposit the fungicide in the fibres of the fabric, and coating the dried fabric with a rubber composition.

In testimony whereof we affix our signatures.

FRANK A. McDERMOTT.  
FOREST J. FUNK.

15

50

60

65